

**3,171,812**  
**ANTIPLUGGING AGENTS FOR HYDROXY**  
**STEARATE GREASES**

Alcide C. Horth, Sarnia, Ontario, and Warren C. Patterson, Mooretown, Ontario, Canada, assignors to Esso Research and Engineering Company, a corporation of Delaware  
No Drawing. Filed July 25, 1960, Ser. No. 44,857  
5 Claims. (Cl. 252—40)

This invention relates to metal hydroxy stearate grease compositions adapted to be dispensed by centralized lubrication systems. Particularly, the invention relates to calcium, lithium, or calcium-lithium hydroxy stearate greases containing a small amount of additive to prevent plugging of small diameter feed lines in centralized lubrication systems.

Calcium, lithium and mixed calcium-lithium hydroxy stearate greases are well known in the art and in general, have excellent shear stability and non-bleeding characteristics. However, when these greases are subjected to forced feeding under high pressure through narrow diameter orifices or lines such as are encountered in centralized lubrication systems, there is a tendency for the grease to form hard solid deposits which plug the feed lines of the system. It has been found that by the addition of a small amount of certain agents to the grease, that its resistance to plugging is greatly increased.

The antiplugging agents found particularly useful are water, glycerine, and polyalkylene glycols such as polyethylene glycol of 200 to 7,000, preferably 700 to 3,000 molecular weight. It has been further found that a combination of 0.5 to 1.0 part by weight of water per part by weight of glycerine is more effective than a like amount of either water or glycerine. While these materials have been previously used in greases, it is believed that their use and mode of use in the hydroxy stearate greases of the invention is new.

Thus, water has been previously used in low temperature grease systems, particularly in simple calcium soap grease, in order to give the grease a fibrous nature and hold it together. One advantage of the hydroxy stearate greases, particularly calcium hydroxy stearate greases, is that water is not necessary for this purpose, since the hydroxy portion of the molecule acts as a linking agent and imparts fibrousness to the grease. As a result, hydroxy stearate greases in practice are completely dehydrated during preparation and it is unconventional to form a finished 12-hydroxy stearate grease containing free water.

Glycerine and polyalkylene glycols are known as structure modifiers. Thus, Bondi, in U.S. Patent 2,475,589, describes the addition of glycerine, polyalkylene glycols and naphthenates to greases thickened with a mixture of soaps of hydroxy stearic acid and hydrogenated fish oil fatty acids to minimize bleeding and improve shear stability. However, calcium, calcium-lithium or lithium 12-hydroxy stearate greases (absent the fish oil acid soap) do not require structure modifiers as taught by Bondi. In addition, while Bondi had his additives present during the cooling operation, i.e. present in the melted grease, the process of the present invention preferably involves adding the additives to a cold or slightly warm grease. By this latter method, the loss in hardness (i.e. yield) and color degradation which frequently occurs when glycerol and polyalkylene glycols are present in grease at high temperatures is avoided.

The grease compositions of this invention will therefore comprise a major amount of lubricating oil, about 5 to 30, preferably 5 to 15 wt. percent of a metal hydroxy stearate and about 0.1 to 3.0, preferably 0.2 to 1.0 wt. percent of antiplugging agent.

The metal component of the hydroxy stearate can be lithium or calcium or a mixture thereof.

The lubricating oil is preferably a mineral lubricating oil although synthetic oils such as diesters may be used.

5 Conventional additives can also be added, including oxidation inhibitors such as phenyl-alpha-naphthylamine; rust preventives such as sodium nitrite; tackiness agents such as polyisobutylene, dyes, auxiliary thickeners and the like.

10 The antiplugging additives can be simply added to the finished grease composition by mixing. Preferably, these additives are added during the cooling cycle of the preparation of the grease, i.e. at temperatures below the melting point of the hydroxy stearate soap, e.g. below 200° F.

15 A Trabon centralized lubrication system was used in order to test the plugging characteristics of the greases of the invention. This system included a pump circulating the grease from a reservoir through small diameter feed tubes and back to the reservoir. The number of hours of operation before plugging of the system was determined.

20 The invention will be further understood by reference to the following examples which include a preferred form of the invention.

*Example I*

Two base greases were used in the experiments: Grease A consisted of mineral lubricating oil thickened with 9 wt. percent of calcium-lithium 12-hydroxy stearate thickener in a weight ratio of calcium hydroxy stearate to lithium hydroxy stearate of 4:1. Grease B consisted of mineral lubricating oil thickened with 8.7 wt. percent of calcium 12-hydroxy stearate and containing about 9.25 wt. percent of extreme pressure additives. To these greases were added varying amounts of water, glycerine and polyethylene glycol of 1500 molecular weight. This addition was made by simply mixing the water, glycerine or polyethylene glycol into the grease at room temperature. The compositions were then tested in the centralized lubrication system previously described above and the time required for plugging of this system recorded. The compositions tested and the results obtained are summarized in the following table:

45 **EFFECT OF ANTIPLUGGING ADDITIVES ON GREASE PERFORMANCE IN A TRABON CENTRALIZED LUBRICATION SYSTEM**

| Greases       | Antiplugging Additives                      | Time Necessary for Plugging (Hours) |
|---------------|---------------------------------------------|-------------------------------------|
| Grease A..... | None.....                                   | 48.78                               |
| Do.....       | 0.4% Water.....                             | 165                                 |
| Do.....       | 0.5% Glycerine.....                         | 144                                 |
| Do.....       | 0.9% Glycerine.....                         | 264                                 |
| Do.....       | 0.25% Polyethylene Glycol of 1,500 mol. wt. | 720+                                |
| Do.....       | 0.4% Water, 0.5% Glycerine.....             | 720+                                |
| Grease B..... | None.....                                   | 354                                 |
| Do.....       | 0.5% Glycerine.....                         | 720+                                |
| Do.....       | 0.4% Water, 0.5% Glycerine.....             | 720+                                |

60 As seen by the preceding table, water, glycerine and polyethylene glycol were all effective in preventing plugging. The maximum pressures upon the grease during testing in the Trabon lubricator were about 2500 p.s.i.g., 65 while the smallest orifices through which the grease was passed were about  $\frac{1}{32}$  inch diameter.

In sum, the present invention relates to calcium, lithium and calcium-lithium greases prepared from 12-hydroxy stearic acid and containing a small amount of antiplugging agent. This grease is particularly adapted for use under high pressures, e.g. 500 to 5,000 p.s.i.g., and in small diameter lines, e.g.  $\frac{1}{32}$  to  $\frac{1}{4}$  inch lines or orifices.

What is claimed is:

1. A lubricating grease suitable for use in centralized lubrication systems under high pressure comprising a major amount of mineral lubricating oil, about 5 to 30 wt. percent of a grease thickener consisting essentially of metal hydroxy stearate, and about 0.1 to 3.0 wt. percent of a material selected from the group consisting of glycerine, polyethylene glycol of 700 to 7,000 molecular weight, and mixtures consisting of water and glycerine in a weight ratio of from 0.5-1.0:1, wherein said metal is selected from the group consisting of calcium, and mixtures of calcium and lithium wherein said calcium is present in a major molar amount and wherein all of said material which is present was added to a mixture of said oil and said stearate at a temperature below 200° F. 15

2. A grease composition according to claim 1, wherein said material is glycerine.

3. A grease composition according to claim 1, wherein said material is a mixture of water and glycerine.

4. A grease composition according to claim 1, wherein said material is polyethylene glycol of 700 to 3,000 molecular weight.

5. A lubricating grease according to claim 1, wherein

the amount of said metal hydroxy stearate is 5 to 15.0 wt. percent, the amount of said material is 0.2 to 1.0 wt. percent and said metal consists of calcium.

#### References Cited in the file of this patent

#### UNITED STATES PATENTS

|           |                  |                |
|-----------|------------------|----------------|
| 2,339,715 | McOmie et al.    | Jan 18, 1944   |
| 2,397,956 | Fraser           | Apr. 9, 1946   |
| 2,450,254 | Puryear et al.   | Sept. 28, 1948 |
| 2,607,734 | Sproule et al.   | Aug. 19, 1952  |
| 2,846,394 | Brunstrum et al. | Aug. 5, 1958   |
| 2,878,186 | Liddy            | Mar. 17, 1959  |
| 2,898,298 | Zweifel et al.   | Aug. 14, 1959  |
| 2,929,782 | Sproule et al.   | Mar. 22, 1960  |

#### FOREIGN PATENTS

|         |           |                |
|---------|-----------|----------------|
| 134,363 | Australia | Sept. 21, 1947 |
| 579,995 | Canada    | July 21, 1959  |

#### OTHER REFERENCES

The Manufacture and Application of Lubricating Greases, Boner, Reinhold Publication Corp., New York (1954), pages 43-44.